

# United States Patent

Di Russo et al.

[15] **3,706,606**  
[45] **Dec. 19, 1972**

[54] **THERMOMECHANICAL TREATMENT  
PROCESS FOR HEAT TREATABLE  
ALUMINIUM ALLOYS**

|           |        |                     |          |
|-----------|--------|---------------------|----------|
| 3,454,435 | 7/1969 | Jacobs.....         | 148/12.7 |
| 2,249,349 | 7/1941 | Deutsch .....       | 148/12.7 |
| 3,198,676 | 8/1965 | Sprowls et al. .... | 148/159  |

[72] Inventors: **Ettore Di Russo; Mario Conserva,**  
both of Novara, Italy

Primary Examiner—W. W. Stallard

Attorney—Stevens, Davis, Miller & Mosher

[73] Assignee: **Societa per L'Esercizio dell'Istituto  
Sperimentale dei Metalli Leggeri  
S.p.A., Milan, Italy**

[57] **ABSTRACT**

[22] Filed: **April 14, 1970**

Heat treatable aluminum alloys of increased mechanical strength are produced by submitting the alloy to a solution and quenching treatment followed by a combination of plastic deformations and precipitation hardening, including a first aging treatment at a temperature not higher than 200°C, a plastic deformation and then a further aging at a temperature not lower than the first, the combination for deformations and hardenings being a cycle repeatable on the alloy.

[21] Appl. No.: **28,514**

[30] **Foreign Application Priority Data**

Feb. 10, 1970 Italy.....20,399 A/70

[52] **U.S. Cl.....148/12.7**

[51] **Int. Cl.....C22f 1/04**

[58] **Field of Search.....148/127, 159**

**3 Claims, No Drawings**

[56] **References Cited**

**UNITED STATES PATENTS**

2,083,576 6/1937 Nock.....148/159

## THERMOMECHANICAL TREATMENT PROCESS FOR HEAT TREATABLE ALUMINIUM ALLOYS

The present invention concerns a thermomechanical process particularly suitable to achieve a remarkable increase in the mechanical strength of semifinished heat treatable aluminum alloys without negatively affecting the secondary properties thereof.

This invention particularly comprises specific thermomechanical treatments specially suitable for aluminum alloys of the system Al-Zn-Mg; Al-Zn-Mg-Cu; Al-Cu; Al-Cu-Mg; Al-Cu-Mg-Si; Al-Si-Mg; said alloys being particularly useful for the aeronautical and motor industries as well as, more extensively for constructional parts requiring high mechanical strength. The improvements in the alloy properties can be attained, according to the present invention, through thermomechanical cycles based on suitable combinations of plastic deformations and hardening by precipitation; by these treatments it is in fact possible to induce in the materials a condition of super-hardening related to the combined effect of the hardening phases and of a stable structure of a dislocation network induced by the deformation.

The thermomechanical cycle according to the present invention substantially differentiates from the combined cycles deformation and aging suggested for heat treatable Al alloys by prior art disclosures both in consequence of the different sequence of the various phases making up a thermomechanical cycle and also owing to the particular temperatures used for some intermediate phases; the sequence of phases according to this invention allows in fact one to obtain, particularly for some kinds of alloys, better combinations of static strength and secondary characteristics by virtue of the fact that a real super-hardening condition, unobtainable through the known thermomechanical cycles, is induced in said alloys.

Particularly, the known combined treatments so far used for Al alloys of the systems Al-Cu-MG, Al-Cu, Al-Si-Mg and Al-Zn-Mg-Cu do not lead to such results as are obtainable through the herein proposed sequence of cycles, since said known treatments do not induce any superhardening condition characterized by high structural stability.

An object of the present invention is to provide a particular thermomechanical process suitable to induce in said heat treatable Al alloys a super-hardening such as to grant them remarkable improvements in their static strength characteristics without negatively influencing the other properties of said alloys.

Another object of the present invention is to provide a process which, by establishing such a super-hardening, succeeds in improving some secondary characteristics of said alloys without significantly altering other secondary characteristics while always producing a static mechanical strength not below but often above that obtainable on the same alloys through traditional treatments.

These objects are advantageously reached through a thermomechanical process suited to induce in the heat treatable Al alloys a super-hardening characterized by its high structural stability, said process according to this invention comprising submitting said aluminum alloys, preferably in the form of bars, sheets plates and like preformed shapes to a solution and quenching (T)

5 treatment in water or blast air, followed by a combination of plastic deformations and precipitation hardenings including: a first aging treatment (A<sub>1</sub>) at temperature below 200°C, for a time not longer than 50 hours, a plastic deformation (H), preferably a thickness or section reduction and then a further aging (A<sub>2</sub>) at a temperature and for a time preferably not smaller than the ones used for said first aging treatment, said combination of deformations and hardenings (A<sub>1</sub>HA<sub>2</sub>) making up a treatment cycle repeatable — at temperatures and for times preferably different from the mentioned ones — on the same alloy sample, for further improving its mechanical properties.

10 More particularly said thermomechanical process comprises for the alloys having Cu as the main alloying element, a plastic deformation (H) not below 5 percent, after said quenching treatment (T). The general scheme of the thermomechanical treatment which is 15 within the scope of this invention and applicable to heat treatable Al alloys, is of the type: TA<sub>1</sub>HA<sub>2</sub>; TA<sub>1</sub>HA<sub>2</sub>HA<sub>3</sub>... or type THA<sub>1</sub>HA<sub>2</sub>; THA<sub>1</sub>HA<sub>2</sub>HA<sub>3</sub>... wherein

20 T stands for a solution (performed at various temperatures and for different heating times) and quenching carried out in various media and at various cooling rates,

25 A<sub>1</sub> represents an aging treatment developed (through one or more stages, at various temperatures and for different heating times) till obtaining in the material a distribution of precipitated or pre-precipitated zones, coherent and/or semi-coherent, with a stability degree such as to obtain the effectiveness of the selected thermomechanical cycle in its following stages,

30 H stands for a plastic deformation brought about, with cold or warm processing, in a way and at values such as to let the material acquire high density and homogeneous distribution of dislocations network while retaining also, after its deformation, the possibility of a following hardening due to aging.

35 A<sub>2</sub>A<sub>3</sub>... etc. represent intermediate or final steps of aging carried out at selected temperature and through suitable times, in such a way as to induce in the material a composed structure of dislocations and of a final precipitation hardening as favorable as possible for the final characteristics wished for the material.

40 It has in practice been found that any semifinished product of heat treatable Al alloy of commercial type can be advantageously treated with the process according to this invention; it has been also found that the best results are obtained when the concerned process is applied to semifinished materials coming from ingots or plates submitted to particularly strong cycles of homogenization, as well as when this process is applied to semifinished material coming from alloys prepared with high purity Al and from alloys containing particular additional elements, mainly when said semifinished materials are submitted to strong homogenization cycles.

45 The thermomechanical process according to this invention is particularly suitable for treating Al alloys of the type: Al-Zn-Mg; Al-Zn-Mg-Cu; Al-Cu, Al-Cu-Mg; Al-Cu-Mg-Si; Al-Si-Mg.

To better evidence the results obtainable through this process, some examples of treatment of Al alloys are given hereinafter for illustration only and are not to be construed as limiting of the invention in scope.

In addition to the treatment of this invention, known treatments are also reported in said examples, and included tables, to better evidence the remarkable improvements obtained in the final characteristics of the materials.

It is also to be noted that in said examples the known treatments are carried out using the best known conditions for obtaining the best results in properties, so that these results can be compared with the results of the cycles according to this invention.

In said examples:

$R_m$  is the mechanical tensile strength, in  $\text{kg}/\text{mm}^2$

$R_p$  (0.2) is the permanent deformation limit load, in  $\text{kg}/\text{mm}^2$

$A_5$  stands for the ultimate elongation, in percent.

#### EXAMPLE 1

Five rolled sheets (thickness = 5 mm) of commercial alloy with composition Al—5.1% Zn — 1.1% Mg — 0.14% Cr — 0.21% Mn — 0.12% Zr — 0.12% Fe — 0.10% Si were submitted to quenching (after pre-heating at 460°C for 1 hour) in water at room temperature, every sheet treated in this way being afterwards submitted to a different thermal or thermomechanical cycle. Said cycles, each for every sheet, were as follows:

TA (known cycle - isothermal (one step) aging)

TA<sub>1</sub>A<sub>2</sub> (known cycle -di-isothermal (two step) aging)

THA<sub>1</sub>A<sub>2</sub> (known cycle )

TA<sub>1</sub>A<sub>2</sub>H (known cycle )

TA<sub>1</sub>HA<sub>2</sub> (cycle according to this invention)

wherein H represents a 20 percent reduction in thickness obtained through rolling at room temperature, parallel to the original rolling direction

Mechanical tensile tests were carried out along the rolling direction corresponding to the hardness peaks of every treatment cycle and the ascertained results are shown in the following table 1.

TABLE 1

| Cycle                            | Treatment                      |                                   |                                |                                   | Mechanical Properties                |                                            |                     |  |
|----------------------------------|--------------------------------|-----------------------------------|--------------------------------|-----------------------------------|--------------------------------------|--------------------------------------------|---------------------|--|
|                                  | A <sub>1</sub><br>Temp<br>(°C) | A <sub>1</sub><br>Time<br>(hours) | A <sub>2</sub><br>Temp<br>(°C) | A <sub>2</sub><br>Time<br>(hours) | R <sub>m</sub><br>Kg/mm <sup>2</sup> | R <sub>p</sub> (0.2)<br>Kg/mm <sup>2</sup> | A <sub>5</sub><br>% |  |
| TA <sub>1</sub>                  | 100                            | 200                               | —                              | —                                 | 40.1                                 | 34.8                                       | 16.5                |  |
| TA <sub>1</sub> A <sub>2</sub>   | 100                            | 10                                | 130                            | 22                                | 38.4                                 | 33.7                                       | 17.0                |  |
| THA <sub>1</sub> A <sub>2</sub>  | 100                            | 10                                | 130                            | 22                                | 34.9                                 | 31.8                                       | 13.3                |  |
| TA <sub>1</sub> A <sub>2</sub> H | 100                            | 10                                | 130                            | 22                                | 44.8                                 | 43.2                                       | 6.8                 |  |
| TA <sub>1</sub> HA <sub>2</sub>  | 100                            | 10                                | 100                            | 120                               | 44.3                                 | 42.2                                       | 12.4                |  |

This table clearly evidences that cycle TA<sub>1</sub>HA<sub>2</sub>, according to the present invention, gives the best results and particularly the highest combination of strength and ductility.

#### EXAMPLE 2

Two portions of commercial plate of 35 mm thickness with composition Al — 4.35% Zn — 2.06% Mg — 0.15% Cr — 0.22% Mn — 0.10% Zr — 0.17% Fe — 0.15% Si were submitted to a solution treatment at

60

65

460°C for two hours under steady conditions; one sample was then drastically quenched in cold water (T), while the other was quenched in a stream of air (Ta.v.).

Three samples of the first portion previously treated in cold water, were submitted to thermal and thermomechanical (one for every specimen) treatments according to the following cycles: TA<sub>1</sub>A<sub>2</sub> — TA<sub>1</sub>HA<sub>2</sub> — TA<sub>1</sub>HA<sub>2</sub> while three further samples of the second portion, previously treated in an air stream, were submitted to treatments (one for every sample) of the type: Ta.v.A<sub>1</sub>A<sub>2</sub> — Ta.v.A<sub>1</sub>HA<sub>2</sub> — Ta.v.A<sub>1</sub>HA<sub>2</sub>.

H represents a 20 percent plastic deformation (thickness reduction) brought about on each of the six samples by rolling them, at room temperature, parallel to the direction of the original working.

Specimens were taken from the long transverse direction of said samples, to ascertain mechanical characteristics ( $R_m$ ,  $R_p$  and  $A_5$ ) and stress corrosion resistance (by continuous dip in a 3% NaCl solution buffered at pH = 5.2, being the tensile stress applied to the specimen equal to 75 percent of  $R_p$  (0.2)). The following Table 2 shows the results which were obtained:

TABLE 2

| Cycle                               | Treatment                      |                                   |                                |                                   | Mechanical Properties                   |                                               |                     | Average time for stress corrosion failure Hours |
|-------------------------------------|--------------------------------|-----------------------------------|--------------------------------|-----------------------------------|-----------------------------------------|-----------------------------------------------|---------------------|-------------------------------------------------|
|                                     | A <sub>1</sub><br>Temp<br>(°C) | A <sub>1</sub><br>Time<br>(hours) | A <sub>2</sub><br>Temp<br>(°C) | A <sub>2</sub><br>Time<br>(hours) | R <sub>m</sub><br>(Kg/mm <sup>2</sup> ) | R <sub>p</sub> (0.2)<br>(Kg/mm <sup>2</sup> ) | A <sub>5</sub><br>% |                                                 |
| TA <sub>1</sub> A <sub>2</sub>      | 100                            | 10                                | 130                            | 22                                | 43.4                                    | 40.1                                          | 7.7                 | 88                                              |
| TA <sub>1</sub> HA <sub>2</sub>     | 100                            | 10                                | 130                            | 6                                 | 45.0                                    | 43.0                                          | 7.5                 | 113                                             |
| TA <sub>1</sub> HA <sub>2</sub>     | 100                            | 10                                | 130                            | 22                                |                                         | 40.8                                          | 6.8                 | 208                                             |
| Ta.v.A <sub>1</sub> A <sub>2</sub>  | 100                            | 10                                | 130                            | 22                                | 40.6                                    | 36.4                                          | 8.0                 | >1000                                           |
| Ta.v.A <sub>1</sub> HA <sub>2</sub> | 100                            | 10                                | 130                            | 6                                 | 42.5                                    | 40.5                                          | 6.8                 | >1000                                           |
| Ta.v.A <sub>1</sub> HA <sub>2</sub> | 100                            | 10                                | 130                            | 22                                | 40.9                                    | 38.5                                          | 6.5                 | >1000                                           |

The table clearly evidences that both thermomechanical cycles TA<sub>1</sub>HA<sub>2</sub> and Ta.v.A<sub>1</sub>HA<sub>2</sub> being within the present invention, lead to remarkable improvements.

In case of water cooling the stress corrosion resistance is improved without involving any decrease in the mechanical properties of the material. In case of air stream/cooling a stress corrosion resistance equal to the one attained through known treatments is maintained but the mechanical properties are improved.

#### EXAMPLE 3

Two extruded rod portions (diameter = 15.2 mm) of commercially produced alloy consisting of Al — 5.07% Zn — 0.96% Mg — 0.14% Cr — 0.22% Mn — 0.12% Zr — 0.13% Fe — 0.10% Si were submitted to quenching (after preheating for 2 hours at 460°), in water at room temperature and subsequently underwent two different thermal and thermomechanical cycles (a cycle different for every rod portion) of the type TA<sub>1</sub>A<sub>2</sub> and TA<sub>1</sub>HA<sub>2</sub>, wherein H stands for a 20

percent deformation given by drawing at 25°C abt. Some specimens were taken from the two portions treated as above, and submitted to mechanical tensile strength tests and rotating cantilever fatigue tests (un-notched specimens): the specific results obtained thereby are shown in the following Table 3.

TABLE 3

| Cycle                           | Treatment              |              |          |                        | Mechanical properties |                          |                                | Fatigue characteristics |                         |                                              |
|---------------------------------|------------------------|--------------|----------|------------------------|-----------------------|--------------------------|--------------------------------|-------------------------|-------------------------|----------------------------------------------|
|                                 | A <sub>1</sub><br>(°C) | Temp<br>(°C) | H<br>(%) | A <sub>2</sub><br>(°C) | Temp<br>(°C)          | Rm<br>Kg/mm <sup>2</sup> | Rp (0.2)<br>Kg/mm <sup>2</sup> | A <sub>5</sub><br>(%)   | Number of<br>cycles (n) | Breaking<br>stress (σ)<br>Kg/mm <sup>2</sup> |
| TA <sub>1</sub> A <sub>2</sub>  | 100                    | 12           | —        | 150                    | 12                    | 43.7                     | 39.9                           | 10.2                    | 10 <sup>5</sup>         | 30.0                                         |
|                                 |                        |              |          |                        |                       |                          |                                |                         | 10 <sup>5</sup>         | 24.0                                         |
|                                 |                        |              |          |                        |                       |                          |                                |                         | 10 <sup>7</sup>         | 21.5                                         |
|                                 |                        |              |          |                        |                       |                          |                                |                         | 10 <sup>8</sup>         | 21.0                                         |
| TA <sub>1</sub> HA <sub>2</sub> | 100                    | 15           | 20       | 115                    | 15                    | 52.4                     | 51.5                           | 6.0                     | 0 <sup>5</sup>          | 31.0                                         |
|                                 |                        |              |          |                        |                       |                          |                                |                         | 10 <sup>6</sup>         | 25.0                                         |
|                                 |                        |              |          |                        |                       |                          |                                |                         | 10 <sup>7</sup>         | 21.5                                         |
|                                 |                        |              |          |                        |                       |                          |                                |                         | 10 <sup>8</sup>         | 20.0                                         |

By the shown data it is seen that the cycle according to this invention highly increases the static strength characteristics, in comparison with a traditional cycle TA<sub>1</sub>A<sub>2</sub>. It is also to be noted that the fatigue characteristics displayed by material treated according to TA<sub>1</sub>HA<sub>2</sub> are substantially analogous to those noticed on material treated according to TA<sub>1</sub>A<sub>2</sub>.

## EXAMPLE 4

Six rolled strips (thickness — 2 mm) of commercially produced Al alloy having composition Al — 5.5% Zn — 2.5% Mg — 1.7% Cu — 0.20% Mn — 0.13% Cr — 0.28% Fe — 0.20% Si — 0.08 Ti — were submitted to quenching in water at room temperature (after pre-heating for one hour at 460°C), followed by various thermal and thermomechanical treatment cycles (a different cycle for every strip) of the type TA<sub>1</sub> — TA<sub>1</sub>A<sub>2</sub> — TA<sub>1</sub>HA<sub>2</sub> — TA<sub>1</sub>HA<sub>2</sub> — TA<sub>1</sub>H — — TA<sub>1</sub>H<sub>1</sub>A<sub>2</sub>H<sub>2</sub>A<sub>3</sub>, wherein H represents a deformation (given by rolling at 25°C and 150°C abt.) produced by working parallel to the original rolling direction, said deformation amounting to 10 percent, 20 percent, 30 percent.

Tensile tests (being the specimen axis parallel to the original rolling direction) were carried out corresponding to the hardness peaks of every treatment cycle and the results obtained appear in the following Table 4:

TABLE 4

| Cycle                                                                       | Treatment              |                 |                       |                        | Mechanical properties |                          |                                |                       |
|-----------------------------------------------------------------------------|------------------------|-----------------|-----------------------|------------------------|-----------------------|--------------------------|--------------------------------|-----------------------|
|                                                                             | A <sub>1</sub><br>(°C) | Temp<br>(hours) | H <sub>1</sub><br>(%) | A <sub>2</sub><br>(°C) | Temp<br>(°C)          | Rm<br>Kg/mm <sup>2</sup> | Rp (0.2)<br>Kg/mm <sup>2</sup> | A <sub>5</sub><br>(%) |
| TA <sub>1</sub>                                                             | 120                    | 24              | —                     | —                      | —                     | 58.5                     | 51.5                           | 13.1                  |
| TA <sub>1</sub> A <sub>2</sub>                                              | 105                    | 6               | —                     | 120                    | 24                    | 59.3                     | 52.3                           | 13.9                  |
| TA <sub>1</sub> HA <sub>2</sub>                                             | 105                    | 6               | 30                    | 105                    | 20                    | 67.0                     | 64.7                           | 7.7                   |
| TA <sub>1</sub> HA <sub>2</sub>                                             | 105                    | 6               | 20                    | 120                    | 8                     | 64.5                     | 60.0                           | 8.0                   |
| TA <sub>1</sub> H                                                           | 120                    | 24              | 20                    | —                      | —                     | 67.1                     | 64.5                           | 4.0                   |
| TA <sub>1</sub> H <sub>1</sub> A <sub>2</sub> H <sub>2</sub> A <sub>3</sub> |                        |                 |                       |                        |                       | 67.4                     | 66.0                           | 7.1                   |

The values used for the last cycle in Table 4, (TA<sub>1</sub>H<sub>1</sub>A<sub>2</sub>H<sub>2</sub>A<sub>3</sub>), were: A<sub>1</sub> = 105°C for 6 hours, H<sub>1</sub> = 20%, A<sub>2</sub> = 105°C for 6 hours, H<sub>2</sub> = 10%, A<sub>3</sub> = 105°C for 15 hours.

## EXAMPLE 5

Two sheets (thickness = 2 mm) were rolled from a chill cast ingot (of 110 mm diameter) (cooled in water after casting) of composition Al — 8.02% Zn — 2.52% Mg — 1.58% Cu — 0.20% Mn — 0.18% Zr — 0.002%

5

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1000

1005

1010

1015

1020

1025

1030

1035

1040

1045

1050

1055

1060

1065

1070

1075

1080

TABLE 6

| Cycle                           | Treatment                      |                 |                                |                 | Mechanical Properties    |                                |                     |
|---------------------------------|--------------------------------|-----------------|--------------------------------|-----------------|--------------------------|--------------------------------|---------------------|
|                                 | A <sub>1</sub><br>Temp<br>(°C) | Time<br>(hours) | A <sub>2</sub><br>Temp<br>(°C) | Time<br>(hours) | Rm<br>Kg/mm <sup>2</sup> | Rp (0.2)<br>Kg/mm <sup>2</sup> | A <sub>s</sub><br>% |
| TA <sub>1</sub>                 | 140                            | 30              | —                              | —               | 47.5                     | 39.3                           | 11.0                |
| TA <sub>1</sub> HA <sub>2</sub> | 140                            | 10              | 140                            | 10              | 49.0                     | 45.2                           | 8.5                 |

This table evidences a remarkable increase in the yield strength as well as a very slight decrease in the elongation attained with the cycle of this invention, in comparison with the results reached through conventional cycle TA<sub>1</sub>; it is therefore quite evident that the combination of properties obtained through the cycle of this invention is superior.

## EXAMPLE 7

Rolled sheets (thickness = 2 mm) of commercially produced alloy Al — 4.5% Cu — 1.5% Mg — 0.56% Mn — 0.33% Fe — 0.14% Si, were submitted, after quenching in room temperature water (previous pre-heating for one hour at 495°C) to various thermal and thermomechanical cycles of the type TA<sub>1</sub> — THA<sub>1</sub> — TA<sub>1</sub>H — TA<sub>1</sub>HA<sub>2</sub> — TH<sub>1</sub>A<sub>1</sub>H<sub>2</sub>A<sub>2</sub> wherein H represents a deformation obtained by rolling at 25°C, parallel to the original rolling direction. The tensile tests (performed with specimen axis parallel to the rolling direction) are shown in following Table No. 7.

TABLE NO. 7

|                                                                      | Treatment                                                                                                                                                          | Rm<br>Kg/mm <sup>2</sup> | Rp (0.2)<br>Kg/mm <sup>2</sup> | A <sub>s</sub><br>% |
|----------------------------------------------------------------------|--------------------------------------------------------------------------------------------------------------------------------------------------------------------|--------------------------|--------------------------------|---------------------|
| Type TA <sub>1</sub>                                                 | A <sub>1</sub> =190°C for 10 hours                                                                                                                                 | 48.6                     | 40.2                           | 14.5                |
| Type THA <sub>1</sub>                                                | A <sub>1</sub> =190°C for 8 hours<br>H = 6% (obtained by cold rolling)                                                                                             | 53.7                     | 52.9                           | 8.1                 |
| Type THA <sub>1</sub>                                                | H=40% (obtained by cold rolling)<br>A <sub>1</sub> = 190°C for 2 hours                                                                                             | 58.2                     | 56.2                           | 6.6                 |
| Type TA <sub>1</sub> H                                               | A <sub>1</sub> = 190°C for 10 hours<br>H = 40% (obtained by cold rolling)                                                                                          | 58.9                     | 56.7                           | 3.5                 |
| Type TA <sub>1</sub> HA <sub>2</sub>                                 | A <sub>1</sub> = 140°C for 8 hours<br>H = 40% (obtained by cold rolling)<br>A <sub>2</sub> = 140°C for 8 hours                                                     | 60.9                     | 54.6                           | 11.4                |
| Type TA <sub>1</sub> HA <sub>2</sub>                                 | A <sub>1</sub> = 140°C for 6 hours<br>H = 20% (obtained by cold rolling)<br>A <sub>2</sub> = 180°C for 4 hours                                                     | 56.1                     | 51.8                           | 12.6                |
| Type TH <sub>1</sub> A <sub>1</sub><br>H <sub>2</sub> A <sub>2</sub> | H <sub>1</sub> = 6% (obtained by cold rolling)<br>A = 140°C for 12 hours<br>H <sub>2</sub> = 20% (obtained by cold rolling)<br>A <sub>2</sub> = 140°C for 20 hours | 58.4                     | 51.9                           | 13.4                |

## EXAMPLE NO. 8

Rolled sheets (thickness = 2 mm) of commercially produced alloy Al — 0.98% Si — 0.73% Mg — 0.62Mn — 0.27% Fe, were submitted (previous quenching car-

ried out after steady preheating of 1 hour at 530°C and cooling in water at room temperature) to various thermal and thermomechanical cycles of the type TA<sub>1</sub> — TA<sub>1</sub>H — TA<sub>1</sub>HA<sub>2</sub> wherein H represents a deformation given by rolling, at 25°C abt., parallel to the original direction of working.

The tensile tests (performed with the specimen axis parallel to the rolling direction) are shown in following Table No. 8.

TABLE 8

|    | Treatment                            | Rm<br>Kg/mm <sup>2</sup>                                                                                         | Rp (0.2)<br>Kg/mm <sup>2</sup> | A <sub>s</sub><br>% |
|----|--------------------------------------|------------------------------------------------------------------------------------------------------------------|--------------------------------|---------------------|
| 15 | Type TA <sub>1</sub>                 | A <sub>1</sub> = 175°C for 8 hours                                                                               | 37.1                           | 34.5                |
| 15 | Type TA <sub>1</sub> H               | A <sub>1</sub> = 160°C for 10 hours<br>H = 20% (obtained by cold rolling)                                        | 37.0                           | 34.0                |
| 20 | Type TA <sub>1</sub> HA <sub>2</sub> | A <sub>1</sub> = 100°C for 50 hours<br>H = 40% (obtained by cold rolling)<br>A <sub>2</sub> = 150°C for 10 hours | 41.0                           | 38.0                |
| 25 | Type TA <sub>1</sub> HA <sub>2</sub> | A <sub>1</sub> = 150°C for 4 hours<br>H = 40% (obtained by cold rolling)<br>A <sub>2</sub> = 150°C for 2 hours   | 43.9                           | 41.8                |

The above given examples clearly demonstrate that the combined thermomechanical treatment (TA<sub>1</sub>HA<sub>2</sub>), being within the present invention surely and always leads to a remarkable increase in the mechanical strength without negatively influencing the secondary properties (in some cases on the contrary improving some of them) such as ultimate elongation, stress corrosion tensile strength, fatigue strength, creep strength etc.

It is obvious that modifications and alternatives with equivalent character can be made while remaining within the spirit and scope of the invention.

What is claimed is:

1. A thermomechanical treatment process for heat treatable aluminum alloys selected from the group consisting of Al-Zn-Mg and Al-Zn-Mg-Cu systems comprising

submitting said alloys in preformed shape to a solution and quenching treatment (T) followed by a combination of plastic deformation and precipitation hardening including:

a first aging treatment (A<sub>1</sub>) at a temperature between 60° and 200°C for times ranging from 2 to 50 hours,

a plastic deformation (H) of between 10 and 30 percent obtained by reducing the thickness of the wrought product and

a further aging treatment (A<sub>2</sub>) at a temperature and for a time at least equal to the conditions employed in said first aging treatment.

2. The process of claim 12 wherein said second aging treatment (A<sub>2</sub>) is carried out at a temperature between 60° and 230°C for times ranging from 2 to 120 hours.

3. The process of claim 12 wherein said combination of deformation and hardenings (A<sub>1</sub>HA<sub>2</sub>) is a cycle repeatable on the same alloy sample at temperatures and for times in the same range as those specified.

\* \* \* \* \*